# EUROPEAN PATENT SPECIFICATION

(11) **EP 0 173 620 B1**
(45) Date of publication and mention of the grant of the patent: **26.04.1989**
(21) Application number: 85401622.7
(22) Date of filing: 09.08.1985
(51) Int. Cl.: G03G 13/22, G03G 13/02, G03G 13/04, G03G 5/04, G03G 5/082, G03G 5/14

(54) **Low field electrophotographic process**
Elektrophotographisches Niederfeldverfahren
Procédé électrophotographique à champ bas

(30) Priority: 20.08.1984 US 642603
(43) Date of publication of application: 05.03.1986
(73) Proprietor: EASTMAN KODAK COMPANY (a New Jersey corporation), Rochester, New York 14650 (US)
(72) Inventor: Borsenberger, Paul M., Rochester New York 14650 (US)
(74) Representative: Parent, Yves

(56) References cited:
- US-A- 4 265 991
- US-A- 4 409 308
- US-A- 4 443 529
- US-A- 4 461 819

## Description

This invention relates in general to electrophotography and in particular to a novel low field electrophotographic process. More specifically, this invention relates to a low field electrophotographic process employing a photoconductive insulating element which exhibits high quantum efficiency at low voltage.

Photoconductive elements comprise a conducting support bearing a layer of a photoconductive material which is insulating in the dark but which becomes conductive upon exposure to radiation. A common technique for forming images with such elements is to uniformly electrostatically charge the surface of the element and then imagewise expose it to radiation. In areas where the photoconductive layer is irradiated, mobile charge carriers are generated which migrate to the surface of the element and there dissipate the surface charge. This leaves behind a charge pattern in nonirradiated areas, referred to as a latent electrostatic image. This latent electrostatic image can then be developed, either on the surface on which it is formed, or on another surface to which it has been transferred, by application of a liquid or dry developer composition which contains electroscopic marking particles. These particles are selectively attracted to and deposit in the charged areas or are repelled by the charged areas and selectively deposited in the uncharged areas. The pattern of marking particles can be fixed to the surface on which they are deposited or they can be transferred to another surface and fixed there.

Photoconductive elements can comprise a single active layer, containing the photoconductive material, or they can comprise multiple active layers. Elements with multiple active layers (sometimes referred to as multi-active elements) have at least one charge-generating layer and at least one charge-transport layer. The charge-generating layer responds to radiation by generating mobile charge carriers and the charge-transport layer facilitates migration of the charge carriers to the surface of the element, where they dissipate the uniform electrostatic charge to light- struck areas and form the latent electrostatic image.

The photoreceptor properties that determine the radiation necessary to form the latent image are the quantum efficiency, the thickness, the dielectric constant, and the existance of trapping. In the simplest case, where trapping can be neglected, the exposure can be expressed as: where E is the exposure in ergs/cm², s the relative dielectric constant, L the thickness in cm, e the electronic charge in esu, λ the wavelength in nm, 0 th quantum efficiency, k a constant equal to 3.2x10⁻¹³, and AV the voltage difference between the image and background area, V,-V_{b}. The quantum efficiency, which cannot exceed unity, represents the fraction of incident photons that are absorbed and result in free electron-hole pairs.

For electrophotographic processes known heretofore, AV is typically 400-500 V. Assuming typical values of e=3.0, \=₅00 nm, and L=₁₀-³ cm, the above equation predicts an exposure energy of 11.8 to 14.7 ergs/cm². This assumes that there is no trapping and is based on the absorbed radiation. In practice, the radiation is not completely absorbed, and the exposure is correspondingly larger. Thus, most photoreceptors require exposures in the range of 20-100 ergs/ cm² to form an electrostatic image. These are equivalent to ASA ratings between 0.1 and 0.02. In contrast, the exposure required to form a latent image in conventional silver halide photography is in the range of 10-² to 10-¹ ergs/cm², or less, and, accordingly, the radiation sensitivity of electrophotography is less than that of convenitonal silver halide photography by a factor of at least 1₀₃.

While increase in electrophotographic sensitivity can be realized by increases in thickness or quantum efficiency, these effects are limited. Increases in photoreceptor thickness tend to result in trapping, which gives rise to a sharp decrease in sensitivity. Since the quantum efficiency cannot exceed unity, increases in efficiency are limited. For the example discussed in the preceeding paragraph, the maximum increase in sensitivity would be a factor of about 5. In practice, absorption and reflection losses, photogeneration efficiencies of less than unity, etc., would limit the increase to probably no more than a factor of about 3. Consequently, if the sensitivity is to be signficantly increased, the magnitude of the voltage difference between the image and background areas must be reduced. Moreover, if the sensitivity is to be increased without a concurrent increase to electrostatic noise, the magnitude of V_{b} must also be reduced, since a reduction in AV without a corresponding reduction in V_{b} results in a very low signal to noise (S/N) ratio.

A reduction in both ΔV and V_{b} requires that the photoreceptor be initially charged to very low voltages, e.g., Vₒ=10 volts. However, with photoconductive elements of both the single-active-layer and multiple-active layer types, the quantum efficiency typically decreases sharply with decreasing voltage. [See D. M. Pai and R. C. Enck, Phys. Rev. 11, 5163, (1975); P. J. Melz, J. Chem. Phys. 57, 1694, (1972); and P. M. Borsenberger and D. C. Hoesterey, J. Appl. Phys. 51, 4248 (1980)]. As a result, electrophotographic processes typically employ a high initial voltage, such as 500 volts, and electrostatic latent image formation tyipcally requires exposures of the order of 20 to 100 ergs/cm².

Thus, the problem of this invention is to provide a high speed electrophotographic process which exhibits minimal electrical noise. The solution to this problem is a novel electrophotographic process in which a photoconductive insulating element is uniformly electrostatically charged and image-wise exposed to activating radiation to thereby form a latent electrostatic image on the surface thereof, said element (1) comprising:
(a) an electrically-conductive support,
(b) a barrier layer overlying the support, and
(c) a photoconductive stratum overlying the barrier layer, characterized in that
   (1) said stratum comprises a layer of intrinsic hydrogenated amorphous silicon in electrical contact with a layer of doped hydrogenated amorphous silicon, said doped layer being very thin in relation to the thickness of the intrinsic hydrogenated amorphous silicon layer, and
   (2) said element is uniformly electrostatically charged to a surface voltage in the range of from 5 to 50 volts, and
   (3) said doped hydrogenated amorphous silicon layer is image-wise exposed to said activating radiation.

The term "activating radiation" as used herein is defined as electromagnetic radiation which is capable of generating electron-hole pairs in the photoconductive insulating element upon exposure thereof.

Use of a very low initial voltage in the process of this invention, that is a voltage in the range of 5 to 50 volts, in combination with use of an amorphous silieon element of the particular structure described herein has been unexpectedly found to provide the desired characteristics of very high electrophotographic sensitivity without excessive electrical noise. The low V_{b} and low V which characterize the process are rendered feasible by the unique electrophotographic properties of the aforesaid element, which provides high quantum efficiency at low voltage.

The invention is hereinafter described in detail with reference to the accompanying drawings in which:
Figure 1 is a logarithmic plot of quantum efficiency versus electric field for a photoconductive insulating element that is useful in the process of this invention and for a control element.
Figure 2 is a V-IogE plotfor the test element and control element of Figure 1.

The preparation of thin films of amorphous silicon, hereinafter referred to as-Si, by the glow discharge decomposition of silane gas, SiH₄, has been known for a number of years. (See, for example, R. C. Chittick, J. H. Alexander and H. F. Sterling, J. Electrochem. Soc., 116, 77, 1969, and R. C. Chittick, J. N-Cryst, Solids, 3, 255, 1970). It is also known that the degree of conductivity and conductivity type of these thin films can be varied by doping with suitable elements in a manner analogous to that observed in crystalline semiconductors. (See, for example, W. E. Spear and P. G. LeComber, Solid State Commun., 17, 1193, 1975). Furthermore, it is widely recognized that the presence of atomic hydrogen plays a major role in the electrical and optical properties of these materials (see, for example, M. H. Brodsky, Thin Solid Films, 50, 57, 1978) and thus there is widespread current interest in the properties and uses of thin films of so-called "hydrogenated amorphous silicon," hereinafter referred to as a-Si(H).

The field of electrophotography is one in which there is extensive current interest in the utilization of thin films of a-Si(H). To date, the art has disclosed a wide variety of photoconductive insulating elements, comprising thin films of intrinsic and/or doped a-Si(H), which are adapted for use in electrophotographic processes. (As used herein, the term "a doped a-Si(H) layer" refers to a layer of hydrogenated amorphous silicon that has been doped with one or more elements to a degree sufficient to render it either n-type or p-type). Included among the many patents describing photoconductive insulating elements containing layers of intrinsic and/or doped a-Si(H) are the following:
Kempter, U.S. Patent 4,225,222, issued September 30, 1980.
Hirai et al, U.S. Patent 4,265,991, issued May 5, 1981.
Fukuda et al, U.S. Patent 4,359,512, issued November 16, 1982.
Shimizu et al, U.S. Patent 4,359,514, issued November 16, 1982.
Ishioka et al, U.S. Patent 4,377,628, issued March 22, 1983.
Shimizu et al, U.S. Patent 4,403,026, issued September 6, 1983.
Shimizu et al, U.S. Patent 4,409,308, issued October 11, 1983.
Kanbe et al, U.S. Patent 4,443,529, issued April 17,1984.
Nakagawa et al, U.S. Patent 4,461,819, issued July 24, 1984.

As hereinabove described, the present invention makes use of a particular type of photoconductive insulating element, characterized by the presence of both doped and intrinsic layers of a-Si(H), in an electrophotographic process in which the element is electrostatically charged to a low surface voltage, that is a voltage in the range of from 5 to 50 volts. More specifically, the photoconductive insulating element utilized in the electrophotographic process of this invention comprises:
(a) an electrically-conductive support, by which is meant a support material which is itself electrically conductive or which is comprised of an electrically-insulating material coated with an electrically-conductive layer,
(b) a barrier layer overlying the support, by which is meant a layer which serves to prevent the migration of charge-carriers from the support into the photoconductive layers of the element, and
(c) a photoconductive stratum overlying the barrier layer which comprises a layer of intrinsic a-Si(H) in electrical contact with a layer of doped a-Si(H) and in which the doped layer is very thin in relation to the thickness of the intrinsic layer.

It is critical to the invention that the photoconductive stratum comprise both an intrinsic a-Si(H) layer and a doped a-(H) layer, since use of an intrinsic a-Si(H) layer alone would not be an effective means of generating the necessary charge carriers when employing a low surface voltage; while use of a doped a-Si(H) layer alone would result in too high a dark conductivity for the element to be useful in the iow field process of this invention. It is also very important that the doped layer be very much thinner than the intrinsic layer, since, if this were not the case, the dark conductivity would be excessively high for use in the low field process of this invention.

It is also critical to the invention that the element be electrostatically charged to a very low surface voltage, that is a voltage in the range of from 5 to 50 volts. Only by the use of such a low voltage is it possible to achieve very high electrophotographic sensitivity-a sensitivity which is so high that the element can be reasonably characterized as a camera-speed material-without the generation of excessive electrical noise. It is this use of very low voltage which specifically distinguishes the process of this invention from conventional electrophotographic processes which utilise much higher voltages.

Photoconductive insulating elements, whether of the single-active-layer or multiple-active-layer types, typically exhibit a quantum efficiency at low voltage which is much less than they exhibit at high voltage. However, the photoconductive insulating elements described herein exhibit a quantum efficiency at low voltage which is substantially the same as that at high voltage. It is this characteristic which renders them especially suitable for use in the novel low field electrophotographic process of this invention.

The elements employed in the process of this invention utilize an electrically-conductive support, and such support can be either an electrically-conductive material or a composite material comprised of an electrically-insulating substrate coated with one or more conductive layers. The electrically-conductive support should be a relatively rigid material and preferably one that has a thermal expansion coefficient that is fairly close so that of a layer of a-Si(H). Particularly useful materials include aluminum, steel, and glass that has been coated with a suitable conductive coating. Preferably, the support is fabricated in a drum or tube configuration, since such configurations are most appropriate for use with a relatively brittle and fragile material such as a-Si(H).

A particularly important feature of the photoconductive insulating element employed in the process of this invention is the barrier layer. It serves to prevent the injection of charge carriers from the substrate into the photoconductive stratum. Specifically, it prevents the injection of holes from the substrate when the photoreceptor is charged to a negative potential, and it prevents the injection of electrons from the substrate when the photoreceptor is charged to a positive potential. Either positive or negative charging can, of course, be used in the process of this invention, as desired. Inclusion of a barrier layer in the element is necessary in order for the element to provide adequate charge acceptance.

A number of materials are known to be useful to form a barrier layer in an amorphous silicon photoconductive insulating element. For example, useful materials include oxides such as silicon oxide (SiO) or aluminum oxide (A1₂0₃). Preferably, the barrier layer is a layer of a-Si(H) which has been heavily doped with a suitable doping agent. The term "heavily doped", as used herein, is intended to mean a concentration of doping agent of at least 100 ppm.

The term "a photoconductive stratum" is used herein to refer to the combination of an intrinsic a-Si(H) layer and a doped a-Si(H) layer in electrical contact therewith. Since the essential requirement is merely that the activating radiation be incident upon the doped layer, the particular order of these layers in the photoconductive stratum is not ordinarily critical. For example, the doped layer can be the outermost layer and the exposure can be from the front side of the element, or the order of the doped and intrinsic layers can be reversed and the exposure can be from the rear side.

The layer of intrinsic a-Si(H) can be formed by processes which are well known in the art. Most commonly, the process employed is a gas phase reaction, known as plasma-induced dissociation, using a silane (for example SiH₄) as the starting material. The hydrogen content of the intrinsic a-Si(H) layer can be varied over a broad range to provide particular characteristics as desired. Generally, the hydrogen content is in the range of 1 to 50 percent and preferably in the range of 5 to 25 percent (the content of hydrogen being defined in atomic percentage).

The layer of doped a-Si(H) can be formed in the same manner as the layer of intrinsic a-Si(H), except that one or more doping elements are utilized in the layer-forming process in an amount sufficient to render the layer n-type or p-type. (Doping elements can also be used in the formation of the intrinsic layer since a layer of hydrogenated amorpho.us silicon, as typically prepared by the plasma-induced dissociation of SiH₄, is slightly n-type and a slight degree of p-doping is typically employed to render it intrinsic). The hydrogen concentration in the doped layer can be in the same general range as in the intrinsic layer.

Many different doping agents are known in the art to be of utility in advantageously modifying the characteristics of a layer of a-Si(H). Included among such doping agents are the elements of Group VA of the Periodic Table, namely N, P, As, Sb and Bi, which provide an n-type layer-that is, one which exhibits a preference for conduction of negative charge carriers (electrons)-and the elements of Group IIIA of the Periodic Table, namely B, Al, Ga, In and TI, which provide a p-type layer-that is one which exhibits a preference for conduction of positive charge carriers (holes). The preferred doping agent for forming an n-type layer is phosphorus, and it is conveniently utilized in the plasma-induced dissociation in the form of phosphine gas (PH₃). The preferred doping agent for forming a p-type layer is boron, and it is conveniently utilized in the plasma-induced dissocation in the form of diborane gas (B₂H₆). '

The concentration of doping agent employed in forming the doped a-Si(H) layer can be varied over a very broad range. Typically, the doping agent is employed in an amount of up to 1,000 ppm in the gaseous composition used to form the doped layer, and preferably in an amount of 15 to 150 ppm. When a doped a-Si(H) layer is utilized as the barrier layer in the element, it is typically a heavily doped layer, for example, a layer formed from a composition containing 500 to 5,000 ppm of the doping agent.

The thickness of the various layers making up the photoconductive insulating elements employed in the process of this invention can be varied widely. The barrier layer will typically have a thickness in the range of from 0.01 to 5 microns (micrometer), and preferably in the range of from 0.05 to 1 micron. The intrinsic a-Si(H) layer will typically have a thickness in the range of from 1 to 50 microns, and preferably in the range of from 3 to 30 microns. The doped a-Si(H) layer will typically have a thickness in the range of from 0.01 to 0.2 microns, and preferably in the range of from 0.02 to 0.1 microns.

The doped a-Si(H) layer must be sufficiently thin to provide the element with a high degree of dark resistivity, generally a dark resistivity of at least 1011 ohm-cm, and most typically in the range of 10¹¹ to 10¹⁴ ohm-cm. While the exact ratio of the thickness of the doped layer to the thickness of the intrinsic layer is not critical, the doped layer is typically very thin in relation to the thickness of the intrinsic layer. It is preferred that the ratio of the thickness of the doped a-Si(H) layer to the thickness of the intrinsic a-Si(H) layer be less than 0.01 and particularly preferred that it be in the range of from 0.001 to 0.005.

As previously indicated, the preferred doping agent for forming an n-type layer is phosphorus, and the preferred doping agent for forming a p-type layer is boron. These agents are preferably utilized in the doped layer at a concentration of 15 to 150 ppm.

The amount of doping agent utilized needs to be carefully controlled to achieve optimum results. For example, an amount of doping agent which is too low will result in an undesirably low quantum efficiency, while an amount of doping agent that is too great will result in an excessively high dark conductivity.

In addition to the essential layers described hereinabove, the photoconductive insulating elements employed in the process of this invention can contain certain optional layers. For example, they can contain anti-reflection layers to reduce reflection and thereby increase efficiency. Silicon nitride is a particularly useful material for forming an anti-reflection layer, and is advantageously employed at a thickness of 0.1 to 0.5 microns.

In the process of this invention, the photoconductive insulating element is electrostatically charged to a surface voltage of 5 to 50 volts, and most preferably of 10 to 20 volts. Charging to this low voltage provides the basis for a very high speed electrophotographic process. The process is also advantageous in that the element has an extremely fast response time, exhibits sensitometry which is essentially temperature independent, and can be readily adapted to provide panchromatic sensitivity through appropriate control of the hydrogen content.

The invention is further illustrated by the following example of its practice.

A photoconductive insulating element was prepared with the following layers arranged in the indicated order:
(1) a glass substrate,
(2) a vacuum-deposited layer of aluminum,
(3) a barrier layer consisting of a 0.15 micron thick layer of SiO,
(4) a 10 micron thick layer of intrinsic a-Si(H), and
(5) a 0.03 micron thick layer of a-Si(H) which had been doped with phosphorus by incorporating_{'} phosphine gas at a concentration of 100 ppm in the silane composition used to form the layer.

Using a positive surface potential and exposure to activating radiation at a wavelength of 400 nm, the quantum efficiency was determined in relation to the magnitude of the surface potential. (The quantum efficiency is defined as the ratio of the decrease in the surface charge density to the absorbed photon flux, assuming the charge density is related to the surface voltage by the geometrical capacitance). The results are shown in Figure 1, which also provides the results for an otherwise identical control element which did not have the doped a-Si(H) layer. In the figure, which is a logarithmic plot of quantum efficiency (0) versus electric field, the results for the test element of the invention are shown by open circles, while those for the control element are shown by solid circles. As shown in Figure 1, the quantum efficiency of the control element decreased substantially with decreasing surface voltage, while the quantum efficiency of the test element was substantially independent of surface voltage over a wide range of voltages. With both the control and test elements, the quantum efficiency at high voltage was unity. As demonstrated by Figure 1, the thin layer of doped a-Si(H) is a critical component of the photoconductive insulating elements which are useful in the process of this invention, as this layer strongly reduces the field dependence of the photogeneration efficiency and thereby gives rise to the high sensitivity that is observed at low fields.

The exposure dependence of the surface voltage for the control and test elements described above, with an initial potential of 10 volts, is shown in Figure 2. In obtaining these data, the exposure wavelength was 400 nm, the exposure duration was 160 microseconds, and the voltage was sampled 0.5 seconds after the cessation of exposure. As shown by Figure 2, the control element exhibited discharge from V. to VJ2 with an exposoure of 0.29 ergs/cm², corresponding to an ASA rating of about 12, while the test element required only 0.11 ergs/cm², corresponding to an ASA rating of about 30.

## Claims

1. An electrophotographic process in which a photoconductive insulating element is uniformly electrostatically charged and image-wise exposed to activating radiation to thereby form a latent electrostatic image on the surface thereof, said element comprising:
(a) an electrically-conductive support,
(b) a barrier layer overlying said support, and
(c) a photoconductive stratum overlying said barrier layer, characterized in that,
(1) said stratum comprises a layer of intrinsic a-Si(H) in electrical contact with a layer of a doped a-Si(H), said doped a-Si(H) layer being very thin in relation to the thickness of said intrinsic a-Si(H) layer, and
(2) said element is uniformly electrostatically charged to a surface voltage in the range of from 5 to 50 volts, and
(3) said doped a-Si(H) layer is image-wise exposed to said activating radiation.

2. A process as claimed in claim 1 wherein said surface voltage is in the range of from 10 to 20 volts.

3. A process as claimed in either of claims 1 or 2 wherein said doped a-Si(H) layer is doped with an element of Group IIIA or Group VA of the Periodic Table.

4. A process as claimed in any of claims 1, 2 or 3 wherein said doped a-Si(H) layer is doped with phosphorus at a concentration of 15 to 150 ppm.

5. A process as claimed in any of claims 1, 2, 3 or 4 wherein the hydrogen concentration in both said intrinsic a-Si(H) layer and said doped a-Si(H) layer is in the range of 5 to 25 percent.

6. A process as claimed in any of claims 1, 2, 3, 4 or 5 wherein the thickness of said intrinsic a-Si(H) layer is in the range of 3 to 30 microns and the thickness of said doped a-Si(H) layer is in the range of 0.02 to 0.1 microns.

7. A process as claimed in any of claims 1, 2, 3, 4, 5 or 6 wherein the ratio of the thickness of said doped a-Si(H) layer to the thickness of said intrinsic a-Si(H) layer is in the range of from 0.001 to 0.005.

## Patentansprüche

1. Elektrophotographisches Verfahren, in dem ein photoleitfähiges, isolierendes Element gleichförmig elektrostatisch aufgeladen und bildweise aktivierender Strahlung exponiert wird, um dadurch ein latentes elektrostatisches Bild auf der Oberfläche des Elementes zu erzeugen, wobei das Element aufweist:
(a) einen elektrisch leitfähigen Träger,
(b) eine Trennschicht über dem Träger und
(c) eine photoleitfähige Formation über der Trennschicht, dadurch gekennzeichnet, daß
(1) die Formation eine Schicht aus Intrinsic a-Si(H) in elektrischem Kontakt mit einer Schicht aus dotiertem a-Si(H) umfaßt, wobei gilt, daß die dotierte a-Si(H)-Schicht sehr dünn im Verhältnis zur Dicke der Intrinsic a-Si(H)-Schicht ist, daß
(2) das Element gleichförmig elektrostatisch auf eine Oberflächenspannung im Bereich von 5 bis 50 Volt aufgeladen wird, und daß
(3) die dotierte a-Si(H)-Schicht der aktivierenden Strahlung bildweise exponiert wird.

2. Verfahren nach Anspruch 1, in dem die Oberflächenspannung im Bereich von 10 bis 20 Volt liegt.

3. Verfahren nach einem der Ansprüche 1 oder 2, in dem die dotierte a-Si(H)-Schicht mit einem Element aus der Gruppe IIIA oder VA des Periodischen Systems der Element dotiert ist.

4. Verfahren nach einem der Ansprüche 1, 2 oder 3, in dem die dotierte a-Si(H)-Schicht mit Phosphor in einer Konzentration von 15 bis 150 ppm dotiert ist.

5. Verfahren nach einem der Ansprüche 1, 2, 3 oder 4, in dem die Wasserstoffkonzentration sowohl in der Intrinsic a-Si(H)-Schicht wie auch in der dotierten a-Si(H)-Schicht im Bereich von 5 bis 25 Prozent liegt.

6. Verfahren nach einem der Ansprüche 1, 2, 3, 4 oder 5, in dem die Dicke der Intrinsic a-Si(H)-Schicht im Bereich von 3 bis 30 Mikron und die Dicke der dotierten a-Si(H)-Schicht im Bereich von 0,02 bis 0,1 Mikron liegt.

7. Verfahren nach einem der Ansprüche 1, 2, 3, 4, 5 oder 6, in dem das Verhältnis der Dicke von der dotierten a-Si(H)-Schicht zur Dicke der Intrinsic a-Si(H)-Schicht im Bereich von 0,001 bis 0,005 liegt.

## Revendications

1. Procédé électrophotographique dans lequel on charge électrostatiquement un élément isolant photoconducteur et on l'expose à un rayonnement activant afin de former une image latente électrostatique sur la surface dudit élément, ledit élément comprenant:
(a) un support conducteur vis-à-vis de l'électricité
(b) une couche barrière recouvrant ledit support, et
(c) un ensemble de couches photoconducteur recouvrant ladite couche barrière, caractérisé en ce que,
(1) ledit ensemble de couches photoconducteur comprend une couche d'a-Si(H) non dopé en contact électrique avec une couche d'a-Si(H) dopé, ladite couche d'a-Si(H) dopé étant très mince par rapport à ladite couche d'a-Si(H) non dopé, et
(2) ledit élément est chargé électrostatiquement uniformément à un potentiel de surface compris entre 5 et 50 volts, et
(3) ladite couche d'a-Si(H) dopé est exposée à un rayonnement activant.

2. Procédé selon la revendication 1, dans lequel le potentiel de surface est compris entre 10 et 20 volts.

3. Procédé selon la revendication 1 ou 2, dans lequel ladite couche d'a-Si(H) dopé est dopée avec un élément du groupe III A ou V A de la classification périodique.

4. Procédé selon l'une quelconque des revendications 1 à 3, dans lequel ladite couche d'a-Si(H) dopé est dopée avec du phosphore à une concentration de 15 à 150 ppm.

5. Procédé selon l'une quelconque des revendications 1 à 4, dans lequel la concentration en hydrogène dans chacune desdites couches d'a-Si(H) non dopé et d'a-Si(H) dopé est comprise entre 5 et 25 pour cent.

6. Procédé selon l'une quelconque des revendications 1 à 5, dans lequel l'épaisseur de ladite couche d'a-Si(H) non dopé est comprise entre 3 et 30 µm et l'épaisseur de ladite couche d'a-Si(H) dopé est comprise entre 0,02 et 0,1 µm.

7. Procédé selon l'une quelconque des revendications 1 à 6, dans lequel le rapport de l'épaisseur de ladite couche d'a-Si(H) dopé à l'épaisseur de ladite couche d'a-Si(H) non dopé est compris entre 0,001 et 0,005.
